

J. Jameson.

Iron & Steel Direct.

No 88,173. Patented Mar 23, 1869.

Fig 1



Fig. 2.



Witnesses

L. H. Aler,

P. T. Dodge

Inventor  
Jacob Jameson  
by Dodge Munn  
his atty

# UNITED STATES PATENT OFFICE.

JACOB JAMESON, OF PHILADELPHIA, PENNSYLVANIA.

## IMPROVEMENT IN THE MANUFACTURE OF IRON AND STEEL.

*Specification forming part of Letters Patent No. 88,173, dated March 23, 1869.*

*To all whom it may concern:*

Be it known that I, JACOB JAMESON, of Philadelphia, in the county of Philadelphia and State of Pennsylvania, have invented certain new and useful Improvements in the Manufacture of Steel and Iron; and I do hereby declare that the following is a full, clear, and exact description thereof, reference being had to the accompanying drawings, making part of this specification, and to the letters of reference marked thereon, like letters indicating like parts wherever they occur.

To enable others skilled in the art to construct and use my invention I will proceed to describe it.

My invention relates to certain improvements in the process of making iron and steel direct from the ore by the use of mineral coal, and in the furnace used for that purpose.

Figure 1 is a transverse horizontal section on the line  $x$   $x$  of Fig. 2. Fig. 2 is a longitudinal vertical section on the line  $y$   $y$  of Fig. 1 of my improved furnace, intended for use with mineral coal.

In this case, I construct the furnace with a series of closed chambers, C, for deoxidizing the ore preparatory to melting the same, as represented in the drawings, this part of the apparatus being the same as that described in my specification, previously filed, and which therefore need not be herein further described. In front of these chambers C, and a little below them, I arrange a puddling-hearth, B, as shown in Fig. 1, in a proper position to readily receive the prepared ore from the chambers C. In front of the hearth B I locate a grate, A, on which the coal is burned, after being prepared as hereinafter explained, there being a door, L, to the fire-grate or box, and another door, I, opening into the puddling-hearth, as represented in Fig. 1, and by blue lines in Fig. 2. Directly in rear of the puddling-hearth B, I locate another or third door, T, which opens direct into the heat-flue D, near the front part of said flue, this being intended for the introduction of blooms for heating them by the same fire that is used to melt the iron.

It should be understood, also, that I use the

hot and damp blast, and also the carbon-chamber described in my patent of March 31, 1868; and that, with the exception of the improvements described in this and my application first previously filed, the furnace is constructed as described in said patent.

In making iron or steel by this process the coal is first prepared by saturating it, in a suitable vessel or box, with brine, or salt and water, and then injecting into and through the mass of coal a jet of steam, by which means the sulphur and other deleterious properties of the coal are, in a great measure, if not wholly, eradicated. The coal, having been thus prepared, is placed on the grate and ignited in the usual manner. The deoxidizing-chambers C are then charged with ore and the fluxes, as heretofore described, and the ore, when sufficiently roasted, is worked along through the chambers, and down upon the puddling-hearth B, where it is melted and worked in the usual manner, the product being wrought-iron; or, by the introduction of carbon produced in the carbon-chambers, as described in my former patent, steel may be produced at will.

If it be desired to produce a superior quality of metal, I use about one-third of pig-iron with two-thirds of the deoxidized metal from the chambers, mixing them on the hearth B. By these means I am enabled to produce either wrought-iron or steel, direct from the ore, and to do so with the use of mineral coal, thus greatly simplifying and cheapening the production of iron and steel.

Having thus described my invention, what I claim is—

1. The herein-described process of making iron or steel direct from the ore, with mineral coal, substantially as set forth.
2. The furnace for treating ores, and producing iron and steel direct therefrom, when constructed and arranged to operate substantially as herein described.

JACOB JAMESON.

Witnesses:

H. B. MUNN,  
W. C. DODGE.